

# United States Patent

[11] 3,615,278

[72] Inventors Zensaku Yamamoto; Susumu Sato; Shujiro Ono; Hiroshi Horiguchi, Muroran, Hokkaido; Shozo Ariga, Setagaya-ku, Tokyo; Shogo Takaishi, Suginami-ku, Tokyo; Hiroshi Sato, Suginami-ku, Tokyo, all of Japan 814,499

[21] Appl. No. 814,499

[22] Filed Mar. 19, 1969

[45] Patented Oct. 26, 1971

[73] Assignee Nippon Steel Corporation Chiyoda-ku, Tokyo, Japan

[32] Priorities Dec. 14, 1963

[33] Japan 38/67288; Dec. 14, 1963, Japan, No. 38/67289; Dec. 14, 1963, Japan, No. 38/67290; Dec. 14, 1963, Japan, No. 38/67291; Sept. 4, 1964, Japan, No. 39/50761

[31] Continuation-in-part of application Ser. No. 417,009, Dec. 9, 1964, now abandoned.

[54] ENAMELING GRADE STEEL AND METHOD OF PRODUCING THE SAME

3 Claims, 15 Drawing Figs.

[52] U.S. Cl. 29/196.1, 75/126, 148/34, 148/39, 164/57, 164/117

[51] Int. Cl. B32b 15/00

[50] Field of Search..... 75/123, 126, 129, 130; 148/12, 39, 12.1, 34, 39; 164/55, 56, 57; 29/186.5, 187.5, 196.1

[56] References Cited

UNITED STATES PATENTS

|           |         |              |          |
|-----------|---------|--------------|----------|
| 2,108,254 | 2/1938  | Devaney..... | 75/58 X  |
| 2,978,765 | 4/1961  | Brown .....  | 164/57 X |
| 3,219,438 | 11/1965 | Poole .....  | 164/55 X |
| 3,392,063 | 7/1968  | Kohler.....  | 148/12   |
| 2,236,504 | 4/1941  | Herty .....  | 75/45    |
| 2,356,450 | 8/1944  | Epstein..... | 75/123   |
| 2,736,648 | 2/1956  | Eckel .....  | 75/123   |

OTHER REFERENCES

I. S. Epstein, et al., New Vanadium Steel for Deep Drawing Sheets, In The Iron Age. p. 158-163. Oct. 12, 1950

Primary Examiner—L. Dewayne Rutledge

Assistant Examiner—Joseph E. Legru

Attorney—McGlew and Toren

**ABSTRACT:** Enameling grade steel ingots or sheets made therefrom, the ingots having a relatively thin outer rimmed layer and a thicker core, the latter being enriched by an alloying metal or metals, especially consisting of Cr, Mn, Al, V, and Ti, which are capable of preventing carbon migration toward the surface or capable of gathering the carbon precipitating in the outer layer toward the core portion during heat treatment or enamel firing above the  $A_1$  transformation point. Also disclosed is a method of making the ingots.



PATENTED OCT 26 1971

3,615,278

SHEET 1 OF 6

FIG. 1



FIG. 2

ANALYSIS OF SLAB OF 140<sup>mm</sup> THICKNESS



PATENTED OCT 26 1971

3,615,278

SHEET 2 OF 6

FIG. 3 (a)



(b)



INVENTORS.

ZENSAKU YAMAMOTO  
SUSUMU SATO  
SHUJIRO ONO  
HIROSHI HORIGUCHI  
SHOZO ARIGA  
SHOGO TAKAISHI  
HIROSHI SATO

BY

*McGraw & Loren*  
ATTORNEYS

PATENTED OCT 26 1971

3,615,278

SHEET 3 OF 6

FIG. 4



(c)



INVENTORS.

ZENSAKU YAMAMOTO  
SUSUMU SATO  
SHUJIRO ONO  
HIROSHI Horiguchi  
SHOZO ARIGA  
SHOGO TAKAISHI  
HIROSHI SATO

BY

McGraw & Loren

ATTORNEYS

PATENTED OCT 26 1971

3,615,278

SHEET 4 OF 6

FIG. 5 (a)



(b)



INVENTORS.

ZENSAKU YAMAMOTO  
SUSUMU SATO  
SHUJIRO ONO  
HIROSHI HORIGUCHI  
SHOZO ARIGA  
SHOGO TAKAISHI  
HIROSHI SATO

BY

*McGraw & Loren*

ATTORNEYS

PATENTED OCT 26 1971

3,615,278

SHEET 5 OF 6



FIG. 6

INVENTORS.

ZENSAKU YAMAMOTO  
SUSUMU SATO  
SHUJIRO ONO  
HIROSHI HORIGUCHI  
SHOZO ARIGA  
SHOGO TAKAISHI  
HIROSHI SATO

BY

*McGraw & Loren*  
ATTORNEYS

PATENTED OCT 26 1971

3,615,278

SHEET 6 OF 6



(a)



(b)



(c)



(d)

FIG. 7

INVENTORS.

ZENSAKU YAMAMOTO  
SUSUMU SATO  
SHUJIRO ONO  
HIROSHI Horiguchi  
SHOZO ARIGA  
SHOGO TAKAISHI  
HIROSHI SATO

BY

*McGraw & Loren*  
ATTORNEYS

## ENAMELING GRADE STEEL AND METHOD OF PRODUCING THE SAME

### CROSS-REFERENCE TO RELATED APPLICATION

This is a continuation-in-part application of Ser. No. 417,009, filed Dec. 9, 1964, now abandoned.

### SUMMARY OF THE INVENTION

The present invention relates to enameling grade steel ingots and sheets made therefrom. The ingots have a relatively thin outer rimmed portion and a thicker core, the latter having incorporated therein predetermined amounts of an alloying metal or metals, which prevent the migration of carbon toward the surface or which are capable of gathering the carbon precipitating in the outer layers toward the core portion during heat treatment or enamel firing above the  $A_1$  transformation point. The invention also relates to a method of producing such steel ingots and steel sheets.

The products made according to the invention exhibit superior properties for enameling purposes and have very satisfactory cold workability. A number of other advantages of the products will be discussed in further detail in the course of the following description.

Prior art low-carbon steel sheets have a great tendency to bend during enameling operations and small projections or craterlike pinholes appear on the enameled surface, thus detrimentally affecting the appearance and quality. These surface defects are usually referred to as "blister." In the surface layer immediately below these blisters, the presence of gathering carbides can be observed. These blisters are caused by escaping CO or CO<sub>2</sub> gas formed in the reaction between oxygen in the enameling chemicals and carbon in the steel.

In a steel high in carbon content, a surface defect called "fish scale" often appears on the enameled surface, which is caused by large amounts of hydrogen escaping from steel during or after the enameling firing process.

As mentioned above, these surface defects are caused by the carbon contained in the steel. Efforts have been made to eliminate these defects. For this purpose, improved enameling grade steels have previously been developed, for example, and extremely low-carbon steel in which the carbon content is maintained below 0.03 percent is produced by a special steel making process or by decarburization annealing. Further, titanium containing steel has been suggested in which the detrimental effects of carbon are alleviated through carbide formation of the added titanium with the carbon.

The above-mentioned improved enameling grade steels have generally good enameling properties, but in lowering the carbon content during the steel making process the oxygen content increases in inverse proportion to the lowering carbon content, thus producing a considerable amount of the non-metallic inclusion in the produced steel. Further, the cold workability of the produced steel sheets is lowered in this manner.

Conventional enameling grade steel, in which carbon is chemically bound by addition of an element such as titanium to form carbides with the carbon, can only be produced in killed form, which results in poor yields. This is so in order to attain alloying conditions in appropriate proportion to the carbon content and oxygen content in the alloying elements and their cold-forming properties are lowered. Moreover, these conventional enameling grade steels are expensive to make. Accordingly, in practice, the ordinary low-carbon rimmed steels are mostly used for general enamels.

Further, when the decarburization is performed in an annealing furnace of the open coil type, the commercial application is limited to steel having less than about 2 mm. thickness, because the decarburization is difficult to perform when the steel is thicker.

Accordingly, it is a primary object of this invention to produce an improved kind of steel suitable for enameling purposes.

Another object is to provide improved steel sheets which can be readily enameled to exhibit superior surface characteristics without having the surface defects referred to.

It is also an object of this invention to provide a process for producing the improved steel and steel sheets.

Generally, it is an object of this invention to improve on the art of enameling grade steel and methods for its production.

5 The inventors have thoroughly investigated the behavior of the carbides just below the steel surface which cause the surface defects during the enameling process of low-carbon steel sheets and have discovered that the surface layer (rimmed layer) of low-carbon steel ingots or hot rolled product obtained therefrom has a lower content of carbon, nitrogen, phosphorus and sulfur than the core portion. This is due to the rimming action during the ingot making. However, when the hot-rolled steel products or the cold-rolled products obtained therefrom are annealed and subjected to enameling firing, the carbon in the steel diffuses and migrates during the annealing and the enameling firing process in a striking degree toward and into the rimmed layer in the surface portion of the steel, as shown in FIG. 3 (b) explained below. Further, it has been discovered that this migration or gathering tendency of the carbon is more pronounced at higher enameling firing temperatures, particularly when the temperature is above the  $A_1$  transformation point.

20 As explained above, in low-carbon rimmed steel, various surface defects occur when the annealing is effected above the  $A_1$  transformation point because the carbon migrates toward the surface and gathers in considerable amounts in the surface layer of the steel. If the annealing is effected below the  $A_1$  transformation point, the migration to and gathering in the 25 surface layer of the carbon is somewhat diminished, but complete prevention of the surface defects on the enameled surface cannot be obtained thereby. The drawability of the steel is also lowered.

30 Based upon the above realization and concept, the enameling grade steel of the present invention contains in its center or core portion predetermined amounts of specific elements effective for preventing diffusion or migration movement of the carbon toward the surface, so that the diffusion movement of the carbon to the surface of the steel sheet during the annealing and enameling firing is prevented. Only incidental amounts of these elements are contained in the rimmed surface layer.

35 In the present invention, an opposite effect is in fact obtained because the carbon is forcibly diffused or caused to migrate toward the core portion during firing and to gather there so that the carbon content in the surface layer of the steel sheet is lower than in the core portion. From a practical point of view, the carbon content in the rimmed surface layer should preferably be lower than about 0.02 percent, whereas the above core will contain 0.04 to 0.15 percent of carbon, whereby the enameling grade steel sheet having excellent surface qualities, superior to those of extremely low-carbon enameling grade steel sheets, is obtained.

40 The results of many experiments indicate that specific alloying metals which are positively effective in causing migration and gathering of the carbon content are chromium, manganese, vanadium, titanium and aluminum.

45 Since these metals lower that austenite-to-ferrite transformation temperature of the steel, the portion of the steel containing appreciable amounts of these elements, i.e., the core portion, has a greater tendency to transform into austenite than the portion containing lesser amounts of such elements, i.e., the rimmed surface layer, during the annealing or during the enameling firing. The steel portion which has transformed to austenite is capable of dissolving much larger amounts of carbon. It is believed that the core portion containing appreciable quantities of such elements has a strong power to attract and collect the carbon content in the steel, for such portion transforms to ferrite only after the remaining portions of the steel have transformed from austenite to ferrite. Accordingly, in steel sheets which contain appreciable amounts of one or more of the enumerated elements mainly in the inner or core portion, the carbon will migrate and gather in the inner portion.

Vanadium, titanium and aluminum, though not effective directly to lower the transformation temperature, are effective to lower the activity of carbon, and thus in the core portion where these elements segregate and accumulate, the content of carbon increases and segregates, whereby the transformation point, in turn, is lowered. Thus, these elements have similar effects as chromium and manganese.

The prior art teachings relating to conventional enameling grade steel do not disclose the incorporation of the alloying metals in the inventive manner, i.e., so that the major portion of these metals is confined to the core portion.

In, for example, producing enameling grade steel sheets containing 0.03 to 0.10 percent of carbon in accordance with this invention, the difference between the content of the inventive alloying metals in the center or core portion and the content of these metals in the surface layer of the steel sheet should be more than about 0.5 percent for chromium and manganese, more than 0.2 percent for titanium and vanadium and more than 0.003 percent for acid soluble aluminum, so as effectively to collect the carbon content predominantly in the center portion of the steel. However, too high a content of these elements tends to harden the steel and to lower the cold workability of the steel. It is, therefore, desirable to maintain the content of these alloying elements as low as possible while still obtaining the desired gathering effect. Experiments have demonstrated that the most desirable range for the content of these elements in the core portion, considering the desired enameling properties and cold workability of the steel, is 0.10 to 0.20 percent for chromium and manganese, 0.05 to 0.15 percent for titanium and vanadium, and 0.005 to 0.002 percent acid soluble aluminum.

In accordance with this invention, the surface defects which are apt to occur during the enameling operation of prior art steels are avoided by preventing the diffusion of carbon to the surface.

Conventional enameling grade steel sheets, in which titanium, niobium, and the like are added, are made from killed steel, and essentially no segregation of carbon in the interior of the sheet takes place. Moreover, titanium, niobium and the like are uniformly distributed in the steel and thus the carbon in steel is diffused uniformly throughout the steel sheet during the annealing, normalizing or enameling firing operation. Accordingly, in the conventional enameling grade steel sheets, the carbon content in the surface layer is equivalent to the average carbon content of the steel.

As will be clearly understood from the above, according to the present invention, it is possible to produce highly satisfactory enameling grade steel sheets with small amounts of the specific elements, which are contained predominantly in the center portion of the steel sheet.

In the steel sheets according to the present invention, a desirable thickness of the surface layer (rimmed layer) is more than about 0.05 mm. This means that the major amount of chromium, manganese, vanadium, titanium and/or acid soluble aluminum is to be present in an inner or core portion which terminates at least 0.05 mm. from the surface. If the surface layer is too thin, it may be destroyed or negatively affected by oxidation during the annealing and normalization prior to the enameling firing proper, or during acid pickling.

Enameling grade steel sheets produced from low-carbon steel in accordance with the invention with an enriched carbon-attracting central or core portion have the following advantages:

1. Fewer defects on the enameled surface.
2. Higher annealing temperatures can be applied to cold rolled products; hence, better cold workability.
3. In the conventional enameling grade steel sheets, in which Ti, Nb, Zr, or Sb is added such elements are uniformly distributed throughout the steel, and the required amount of such elements to be added is considerably larger, which hardens the steel, lowers the cold forming properties and raises the production cost. According to the present invention, however, the specified elements are added only to the center

portion of the steel, and thus the required amount of the elements per unit weight of the steel is much less; hence, improved cold-forming properties and advantages in relation to the production cost.

5. According to the present invention even for a relatively thick sheet above 2.0 mm. an extremely low-carbon surface layer can be obtained, for the carbon content in the steel can be readily collected in the center portion by annealing or normalizing operations.

10. 5. When Ti, Al and V are employed as addition elements the transformation point of the steel from alpha to gamma rises, and thus it is possible to raise the enameling firing temperature as well as to alleviate the possible strain encountered during the enameling firing process.

15. In most cases, enameling grade sheet is used in a drawn form. It is recognized technical problem in the drawing operation that ordinary low-carbon rimmed steel sheets or extremely low-carbon rimmed steel sheets annealed in an open coil system, are susceptible to stretcher strain which is a critical factor for enameling grade steel sheet.

20. Commonly applied measures for preventing the stretcher strain which is encountered during the drawing operation of enameling grade steel sheets are to increase the reduction rate of skin-pass rolling to apply levelling prior to drawing in case of rimmed steel sheets. However, such mechanical treatments, such as by skin-pass rolling or levelling, tend somewhat to lower the cold formability of the steel, require more steps of operation, and cause aging of the steel.

25. 30. The inventive enrichment of the core portion of the sheets with the specified alloying metals effectively overcomes the stretcher strain problem during drawing.

The present invention also relates to a method for casting steel ingots to produce the novel steel composition.

35. After pouring molten steel into an ingot mold, rimming action is maintained for several minutes, whereby a solidified peripheral layer portion is formed. Thereafter, one or several of the specified elements, to wit, manganese, chromium, aluminum, titanium or vanadium in the form of bars, lumps or powder, or alloys of these metals are introduced into the unsolidified portion of the ingot so as to deoxidize and kill the inner portion of the molten steel, as well as to disperse these elements uniformly through the whole volume of unsolidified molten steel. A deoxidizer may also be added. The timing and the method of additions as well as the form of the alloying metals are factors to be considered.

40. 45. The following is an explanation in relation to the production of an ingot having a thickness of 700 to 800 mm. in which the above metals or alloys were added in the form of bars.

50. 55. When the addition element or alloy is added at too early a stage, no satisfactory rimmed layer is formed; hence, satisfactory surface qualities cannot be expected in the steel sheets. On the other hand, when the addition is made at too late a stage, the added alloying elements will be readily distributed uniformly within the core portion. Generally, it is considered that the optimum time of adding the addition element or elements is about 3 to 10 minutes after the pouring, i.e., when the thickness of the solidified outer wall (rimmed layer) has attained about 30 to 70 mm. The ratio of the thickness of the outer surface layer to the thickness of the core should thus preferably be 3:70-1:20.

60. 65. For example, when steel sheets are produced from an ingot of 800 mm. thickness and having a rimmed surface of 40 mm. thickness, sheets of 2 mm. thickness will have a 0.1 mm. thick rimmed surface, and sheets of 1 mm. thickness will have a 0.05 mm. thick rimmed surface.

70. 75. As for the form of the addition elements or alloys, long bars, for example, are preferable in view of the need of distributing the addition elements uniformly in the core portion of the ingot. However, the addition elements or alloys may be incorporated in the form of powder or lumps accommodated in a steel pipe of below 1 mm. wall thickness, which pipe is inserted into the molten core.

In case the addition elements or alloys are introduced in the form of bars, it is obvious that small diameter bars will necessitate a number of such bars to be inserted. On the other hand, large diameter bars result in a greater heat capacity, which causes solidification of a quantity of steel around the bars, and thus the melting of the addition elements or alloys will not take place speedily, uniformly, or continuously, or the bars will often fusion out. Accordingly, the diameter of the bars should be chosen depending in the heat capacity and melting point of the addition elements. However, a diameter of 20 to 30 mm. is generally satisfactory. As for the length of the bars, the use of very short length bars may cause segregation of the addition elements in the upper portion of the ingot only with poor distribution thereof within the core portion. It is thus preferable to employ bars having a length of about 40 percent of the ingot height. Generally, it is important that the placement of the bar in the molten mass of the ingot mold should be effected so as to ensure uniform distribution of the addition elements throughout the unsolidified mass.

The various features of novelty which characterize the invention are pointed out with particularity in the claims annexed to and forming a part of this specification. For a better understanding of the invention, its operating advantages and specific objects attained by its use, reference should be had to the accompanying drawings in which there are illustrated and described preferred embodiments of the invention.

#### BRIEF DESCRIPTION OF THE DRAWINGS

FIG. 1 is a schematic representation of an ingot mold during the addition of Al bars for enriching the core portion of steel in accordance with the invention;

FIGS. 2a-2c show the distribution of soluble aluminum in slabs for cold rolled sheets produced according to the present invention, for ordinary low-carbon rimmed steel sheets and for Al-killed deep drawing steel sheets, respectively;

FIGS. 3a-3b show, respectively, the microstructures of the cold-rolled enameling grade sheets produced according to the present invention and of cold-rolled rimmed steel sheets produced by the conventional method, both annealed at 740° C. for three hours, heated for 4 minutes at 830° C., almost equal to the enameling firing temperature, and quenched in salt water;

FIGS. 4a-4b show, respectively, the manganese distribution in cold-rolled enameling grade sheets produced according to the present invention using manganese as alloying component, and in rimmed steel sheets produced by conventional methods, while FIG. 4c shows the microstructure of the cold-rolled sheets of FIG. 4a as annealed at 720° C. for 6 hours, heated for 4 minutes at 830° C., almost equal to the enameling firing temperature, and quenched in salt water;

FIG. 5a shows the chromium distribution through the thickness of cold-rolled sheets produced according to the present invention using chromium as alloying component;

FIG. 5b shows the microstructure of the same sheet as annealed at 740° C. for 3 hours, heated at 830° C. for four minutes, and quenched in salt water;

FIG. 6 is the microstructure of enameling grade cold-rolled sheets produced according to the present invention using aluminum and chromium in combination as alloying metals, as annealed at 720° C. for 3 hours, heated for 3 minutes at 850° C., almost equal to the enameling firing temperature, and quenched in salt water;

FIG. 7a is a photograph showing the surface appearance of conventional low-carbon rimmed steel sheets on which enameling glaze has been twice applied;

FIG. 7b is a similar photograph as indicated in FIG. 7a showing the surface appearance of a sheet of the present invention to the central portion of which aluminum has been added;

FIGS. 7c and 7d are, respectively, photographs showing the surface appearance of a conventional low-carbon rimmed steel sheet and a sheet of the present invention to the central

portion of which chromium has been added, both sheets having been twice glazed.

#### DETAILED DESCRIPTION OF THE PREFERRED EMBODIMENTS

In FIG. 1, reference numeral 1 represents an ingot mold, 2 is the solidified wall or peripheral surface portion of the steel, 3 is the unsolidified steel mass, and 4 represents several bars of addition elements of relatively small diameter. Since the molten mass in the mold always solidifies from the periphery towards the center, the outer portion 2 solidifies while the core portion is still liquid, so that the bars 4 may be inserted thereinto.

FIG. 2a shows the distribution of acid soluble aluminum in a slab for the cold-rolled sheet produced according to the present invention, in which aluminum in the form of a bar of 26 mm. diameter and 1,400 mm. length has been used. In FIG. 2b, there is represented for comparison purposes the distribution of acid soluble aluminum in a low-carbon rimmed steel while the distribution in A1-killed steel for deep drawing produced according to conventional ingot making methods is shown in FIG. 2c. It is clearly seen from the graphs that the rimmed layer of the steel sheet according to the present invention contains almost no acid soluble aluminum, the acid soluble aluminum being concentrated uniformly in the core portion.

FIG. 4a represents the distribution of manganese in a steel sheet produced according to the present invention in which Fe-Mn alloy granules in a steel pipe of 0.6 mm. wall thickness, 20 mm. diameter, and 1,500 mm. length have been inserted into the core portion. FIG. 4b shows, for comparison purposes, the manganese distribution in low-carbon rimmed steel produced according to conventional ingot making methods. In the sheet of the present invention, as compared with the prior art sheet, manganese is concentrated in the central portion rather than in the surface layer.

The steel of the present invention may be produced in a converter, an open hearth furnace, an electric furnace or any other suitable steel-producing equipment. However, the content of unavoidable elements in the molten steel as teemed, such as Si, P, S, Cu, Ni, Cr, Ti, Nb, V etc. should preferably be maintained as low as possible, although these elements are permitted to be present in the steel in a similar amount as in the ordinary low-carbon rimmed cold-rolled sheets. Thus, it is desirable that the silicon content is not more than 0.01 percent, the contents of phosphorus, sulfur, chromium and nickel are respectively no higher than 0.030 percent, the copper content is not more than 0.10 percent and the contents of niobium, vanadium and titanium are respectively not more than 0.001 percent. Accordingly, the contents of these elements in the surface layer (rimmed layer) of the steel sheet of the present invention are almost equal or somewhat lower than those in the molten steel as teemed, and the contents of these metals do not substantially influence the effects on carbon of the specified alloying elements contained in the central portion of the steel sheets according to the present invention.

When the carbon content in the ladle steel analysis is too low, the oxygen content in the steel remarkably increases, thus increasing nonmetallic inclusions and weakening the rimming action so that a satisfactory rimmed layer is hard to obtain. High carbon content requires larger amounts of the specified alloying elements to be added to the central portion, which, in turn, lowers the cold formability of the sheet. Generally, it is desirable that the carbon content is 0.04 to 0.15 percent.

As for the manganese content in the ladle steel analysis, generally a content of 0.25 to 0.60 percent is desirable in order to prevent red shortness due to FeS. However, for an enameling grade steel, it is desirable that the manganese content is no more than 0.30 percent, for a higher manganese content will increase the strain during the enameling firing process. In this case, the sulfur content should preferably be no more than 0.02 percent.

The hot- and cold-rolling operation of the ingot produced according to the present invention does not affect the essence of the present invention, and can be carried out as easily as in ordinary steel sheet production.

By annealing or normalizing after the hot or cold rolling, carbon in the steel migrates to and gathers in the central portion of the sheet without diffusing and moving to the surface layer so that a surface layer low in carbon content is obtained.

To enhance the activity of the alloying elements thus concentrated in the central portion of the sheet, it is desirable that the annealing or normalizing is effected above 720° C. and the holding time is longer.

Steel products produced from ingots in which the specified alloying metals have been added to the core portion after a rimmed layer of suitable thickness has been solidified have the following advantageous characteristics:

1. they have rimmed layers substantially free from surface defects;
2. surface defects do not appear during the enameling firing;
3. hot and cold workability are good.

The invention will now be described by the following examples, it being understood, however, that these examples are given by way of illustration and not by way of limitation and that many changes may be effected without departing from the scope and spirit of this invention as recited in the appended claims.

#### EXAMPLE 1

An ingot was prepared from top-blown oxygen converter steel in a mold as shown in FIG. 1 under the following conditions:

##### Ladle steel analysis (%):

C: 0.07 Mn: 0.28 Si: 0.01 P: 0.009 S: 0.014

Al added for deoxidation in ladle: 60 g./t.

Pouring temperature: 1,610° C.

Ingot weight: 14,400 kg.

Cross section of ingot: 1,400 mm. wide and 800 mm. thick

Ingot height: 1,800 mm.

Al bars inserted

number: 4 bars

size: 26 mm. diameter and 1,400 mm. length

weight: 7.2 kg. (500 g./t.)

Timing of Al bar insertion: 3 minutes after the pouring.

FIG. 1 shows schematically the position of the inserted Al bars. Molten steel in the ingot mold (1) solidified with rimming action for three minutes and a solidified surface wall (2) of 35 to 40 mm. thickness was formed. The Al bars (4) were then inserted into the unsolidified molten steel portion (3) to a depth of 1,300 mm. from the upper surface of the ingot.

Analysis of cold-rolled sheets of 0.8 mm. thickness produced from the above ingot is as follows:

C: 0.06 percent, Mn: 0.28 percent, Si: 0.01 percent, P: 0.009 percent,

S: 0.015 percent, total N: 0.0021 percent, soluble Al: 0.001 percent in the rimmed layer, 0.008 percent in the core portion.

The mechanical properties of the sheets as annealed at 740° C. for three hours are as follows:

Yield point: 19.2 kg./mm.2, Tensile strength: 33.3 kg./mm.2

Elongation: 46.2 percent, Erichsen value: 11.1 mm., Hardness: HRB 46.2.

For comparison with the product of example 1, rimmed steel was produced from the same charge as stated in example 1 by a conventional ingot making method, i.e. the ingot was prepared in such a way that 800 g. (55 g./t.) of aluminum granules were added uniformly during the pouring for the purpose of controlling the deoxidation. Rimming action was effected for 21 minutes after the pouring. The ingot mold was covered with a small lid (700 kg.).

Analysis and mechanical properties of cold-rolled sheets of 0.8 mm. thickness from the comparison ingot (rimmed steel) are as follows:

C: 0.04 percent, Mn: 0.27 percent, Si: 0.01 percent, P: 0.011 percent,

S: 0.017 percent, total N: 0.0023 percent, soluble Al: 0.001 percent in the rimmed layer, and 0.001 percent in the core layer. Yield point: 23.1 kg./mm.2

Tensile strength: 33.0 kg./mm.2

Elongation: 45.5 percent, Erichsen value: 10.9 mm.

Hardness: HRB 48.5

The above two cold rolled sheets were annealed for three hours at 740° C., heated for four minutes at 830° C., which is almost equal to the enameling firing temperature, and then quenched in salt water. The microstructures of the sheets are shown in FIGS. 3 (a) and (b).

FIG. 3 (b) is the microstructure of the rimmed sheet produced from the comparison ingot. It can be clearly seen that the rimmed layer has a quenched structure of high carbon steel and the central portion (core portion) has a ferrite structure with most of the carbon content being concentrated in the surface layer. By contrast, in FIG. 3 (a) which shows the microstructure of the sheet produced according to the present invention, it is clearly seen that no high carbon phase is present in the surface layer of the sheet, though present in the central portion where much of soluble aluminum is present. The surface layer is thus a ferrite phase, very low in carbon content (presumably less than 0.025 percent of carbon), and the diffusion movement to the surface layer of the carbon content is completely prevented.

Enameling tests were conducted on the above enameling grade steel sheet of the present invention and on the ordinary prior art rimmed steel sheet from the same charge under the following conditions:

|                                |                                              |
|--------------------------------|----------------------------------------------|
| Application of enameling glaze | twice                                        |
| Amount of base glaze           | 3.7 g./dm. <sup>2</sup>                      |
| Firing temperature             | 870° C.                                      |
| Firing period                  | 10 minutes                                   |
| Surface glaze                  | titan white (trade name) of Japan Ferro K.K. |

The photographs of the surface appearance of the two enamelled sheets are shown in FIGS. 7 (a) and (b), respectively. Blisters are visible on the conventional rimmed sheet, but absent on the sheet of the present invention. Parts for gas cooking-pots for rice and gas ranges were made from the sheet of the present invention and the conventional rimmed sheet and subjected to tests for determining their practical usability as enamelwares. The results were that no blisters were detected in any of 200 parts produced from the sheet of the present invention, whereas in case of the conventional rimmed sheet the blister occurrence ratio was 10.5 percent.

Another advantageous feature of the sheet of the present invention is the easiness with which it can be subjected to acid pickling operations. The acid-pickling speed for the sheet of the present invention is about twice as fast as that for the conventional rimmed steel sheet or extremely low-carbon enameling grade steel sheets decarburized by the open coil treatment. This, of course, increases the productivity.

Further, measurements of nonmetallic inclusions in the sheets of the present invention corresponding to all areas of the inner portion of the ingot were carried out for determining purity. A high degree of purity was established.

Conventionally, the addition of deoxidation agents to the ingot mold would impede the floating up or rising of deoxidation products and thus greatly decrease the purity of the products. For this reason, this addition method for deoxidation agents has not been applied in practice in spite of its advantages based on deoxidation in the ingot mold. Surprisingly, the results of the present invention show that the purity of the products of the present invention is strikingly improved as compared with that of sheets produced from ordinary rimmed steel. The amount of nonmetallic inclusions in the products of

the present invention is about half of that in sheets produced from the ordinary rimmed steel. This can be attributed to the following: When aluminum bars or the like alloying metals are inserted into the molten steel rimming in the ingot mold, the aluminum or the like alloying metal melts and a gradual killing effect takes place from within the central portion. While this effect takes place, the convection of molten steel sets in following the rimming action for a considerable time, during which a large amount of scum is seen to float up to the molten steel surface. From this it can be inferred that the oxidation products formed in the inner portion of the molten steel float to the molten steel surface by the action of convection and are absorbed by the scum which has been formed there.

#### EXAMPLE 2

Topblown oxygen converter steel of the following analysis was poured into two ingot molds of the same size as in example 1.

Ladle analysis: C: 0.07%, Si: 0.01%, Mn: 0.26%, P: 0.012%, S: 0.015%, N: 0.0016%

Pouring temperature: 1610°C.

Ladle deoxidation: Al addition: 80 g./t.

After the molten steel in the ingot molds solidified with rimming action for four minutes forming a solidified surface layer, alloy granules of Fe-Ti containing 45 percent of titanium and Fe-V containing 50 percent of vanadium, each packed in a steel pipe of 23 mm. diameter, 1,500 mm. length and 0.6 mm. wall thickness, were respectively inserted into the unsolidified portion of the molten metal in the molds in a similar way as in example 1, whereby Ti and V containing steel ingots were respectively obtained.

Analysis of two hot rolled sheets of 3.2 mm. thickness produced from these ingots is as follows;

|                     | C                                                      | Mn                                                     | P                | S                | N                  |
|---------------------|--------------------------------------------------------|--------------------------------------------------------|------------------|------------------|--------------------|
| Ti-containing sheet | 0.050<br>~ 0.026                                       | 0.27<br>~ 0.23                                         | 0.016<br>~ 0.010 | 0.018<br>~ 0.010 | 0.0026<br>~ 0.0018 |
| V-containing sheet  | 0.045<br>~ 0.026                                       | 0.28<br>~ 0.20                                         | 0.018<br>~ 0.012 | 0.019<br>~ 0.009 | 0.0027<br>~ 0.009  |
|                     | Ti                                                     | V                                                      |                  |                  |                    |
| Ti-containing sheet | trace in surface<br>0.18 - 0.010 in<br>central portion | trace                                                  |                  |                  |                    |
| V-containing sheet  | trace                                                  | trace in surface<br>0.03 - 0.025 in<br>central portion |                  |                  |                    |

These hot-rolled sheets were cold rolled to 0.8 mm. thickness and annealed at 720°C. for 6 hours. Measurements of mechanical properties of the annealed sheets corresponding to the central portion of ingots are shown below:

|                                             | Present Invention   |                     |                                   |
|---------------------------------------------|---------------------|---------------------|-----------------------------------|
|                                             | Ti-containing sheet | Vi-containing sheet | Rimmed Steel Sheet for comparison |
| Erickson value (mm).....                    | 11.40               | 11.58               | 10.78                             |
| C.C.V. (mm).....                            | 36.91               | 37.05               | 37.40                             |
| Yield point (kg/mm <sup>2</sup> ).....      | 16.8                | 16.05               | 20.9                              |
| Tensile strength (kg/mm <sup>2</sup> )..... | 32.7                | 31.7                | 33.0                              |
| Yield rate (percent).....                   | 51.4                | 52.5                | 63.3                              |
| Elongation (percent).....                   | 48.1                | 49.3                | 44.4                              |
| Hardness (HRB).....                         | 38.0                | 39.1                | 42.1                              |

As can be seen from the above table, better Erickson value, C.C.V. value, and elongation value are attained in the Ti-containing and V-containing sheets of the present invention than in the rimmed steel sheet produced from the same melt and heat treated under the same conditions, though the tensile strength value is almost the same. This indicates that the sheets of the present invention have better press workability.

Enameling tests were conducted on the above sheets of the present invention and on the rimmed steel sheet under the same conditions as in example 1. The results were that blisters

were detected in the rimmed steel sheet, but were absent in the sheets of the present invention. The results of tests for determining the usability as enamelwares conducted on 200 parts for gas cooking-pots for rice produced from the sheets of the present invention showed that no blister formation took place in any of the parts.

#### EXAMPLE 3

Topblown oxygen converter steel of the following analysis was prepared:

Ladle analysis: C: 0.06%, Si: 0.01%, Mn: 0.22%, P: 0.008%, S: 0.011%, N: 0.001%

Pouring temperature: 1600°C.

Ladle deoxidation: Al addition: 80 g./t.

This molten steel was poured into an ingot mold under the following conditions:

Ingot weight: 14,400 kg.

Cross section of ingot: 1,400 mm. width and 800 mm.

thickness

Ingot height: 1,800 mm.

After the molten steel in the ingot mold solidified with rimming action for seven minutes and a solidified outer wall of about 60 mm. thickness was formed, alloy granules of Fe-Mn containing 78% of Mn packed in a steel pipe of 20 mm. diameter, 1,500 mm. length and 0.6 mm. wall thickness were inserted into the unsolidified portion of the molten steel in a similar position and manner as the Al bars shown in FIG. 1.

Analysis of cold rolled sheets of 0.8 mm. thickness from the above ingot is as follows:

C: 0.06%, Si: 0.01%, Mn: 0.21% in the rimmed layer, 0.32% in the core portion, P: 0.009%, S: 0.013%, soluble Al: 0.001%.

Distribution of manganese through the thickness of the sheet of the present invention and of ordinary rimmed steel sheets is shown in FIG. 4 (a) and FIG. 4 (b), respectively.

Mechanical properties of the rolled sheet of the present invention as annealed at 720°C. for 6 hours are as follows:

Yield point: 19.3 kg./mm.<sup>2</sup>, Tensile strength: 32.9 kg./mm.<sup>2</sup>, Elongation in 500 mm.: 45.2%, Erichsen value: 10.7 mm., Hardness: HRB 44.2.

FIG. 4 (c) is a photograph showing the microstructure of the annealed sheet which was heated for 4 minutes at 830°C., which is almost equal to the enameling firing temperature, and quenched in salt water. The black portion in the photograph represents the quenched structure of the phase which was austenite at 830°C., and from the Fe-C constitutional diagram it is calculated that this quenched structure contains about 0.2% of carbon. The photograph indicates that the surface layer remained as ferrite even at 840°C. and the carbon content in this portion is below about 0.02 percent, which is the solution limit of carbon in ferrite.

Further, it was confirmed that in the structure of the above annealed sheet, even after being heated at 830°C. and air cooled, there was no segregation of carbon in the surface layer, and the carbon segregation was observed only in the central portion.

Enameling testing was conducted on the above sheet and on a rimmed steel sheet produced from the same charge under the following conditions:

Application of enameling glaze: twice

Amount of base glaze: 3.7 g./dm.<sup>2</sup>

Firing period: 10 minutes

Firing temperature: 870°C.

Surface glaze: titanium white (trade name) of Japan Ferro Co., Ltd.

The results were that blisters were detected in the conventional rimmed steel sheets whereas no blisters were seen in the sheet of the present invention.

The results of tests for determining practical usability of gas cooking-pots and gas ranges produced from the enameled sheet of the present invention showed that no blister formation occurred in any of the 200 test pieces.

## EXAMPLE 4

The molten steel of the same ladle as described in example 1 was poured into an ingot mold of the same size as in example 1. The molten steel was allowed to stand for eight minutes, whereafter a solidified surface wall of about 60 mm. thickness was formed. Alloy granules of Fe-Cr containing 65 percent of chromium packed in a steel pipe of 20 mm. diameter, 1,500 mm. length, and 0.6 mm. wall thickness were then inserted into the molten metal in a similar manner as in example 1.

Analysis of hot rolled sheets of 2.3 mm. thickness produced from the above ingot is as follows:

C: 0.06%, Si: 0.01%, Mn: 0.021%, P: 0.010%,  
S: 0.013%, Cr: 0.011% in the surface layer,  
0.072% in the inner layer.

Distribution of chromium throughout the thickness of the above cold rolled sheet is shown in FIG. 5 (a).

Mechanical properties of cold-rolled sheets of 1.0 mm. thickness, produced from the above hot-rolled sheets, as annealed at 740°C. for 3 hours, are as follows:

Yield point: 21.3 kg./mm.<sup>2</sup>, Tensile strength: 33.0 kg./mm.<sup>2</sup>,  
Elongation: 43.7%, Erickson value: 10.2 mm.  
Hardness: HRB 45.1.

The microstructure of the above annealed sheet as heated at 630°C. for 4 minutes and quenched in salt water in a similar way as in example 1 is shown in FIG. 5 (b).

The sheet of the present invention and a conventional rimmed steel sheet produced from the same charge were subjected to enameling tests under the following conditions:

Glaze applied: H-type glaze of Japan Ferro Co., Ltd.

Amount applied: 3.7 g./dm.<sup>2</sup>

Firing temperature: 870°C.

Firing period: ten minutes

The results were that many blisters were visible in the rimmed steel sheet as shown in FIG. 7 (c), whereas no blister formation was observed in the sheet of the present invention, as shown in FIG. 7 (d).

Tests for determining practical usability were conducted on 500 parts for gas cooking-pots for rice and gas ranges, produced from the sheets of the present invention. These tests indicated that no blisters occurred in any of these parts, whereas tests showed that blister occurrence in the parts produced from the conventional rimmed steel sheet was 13.7 percent.

## EXAMPLE 5

Molten steel containing 0.08% of carbon, 0.01% of silicon, 0.25% of manganese, 0.012% of phosphorus, 0.012% of sulfur (ladle analysis) was poured into an ingot mold of 14.4 ton and rimming action was effected for 3 minutes. Thereafter, 20 kg. of Fe-Cr was added and 1 minute later, Al was added in a similar way as in example 1. Two bars of aluminum were inserted into the center of the unsolidified portion.

Analysis of a cold rolled sheet of 0.8 mm., produced from the above ingot and the mechanical properties of the sheet, as annealed at 720°C. for 3 hours, are as follows:

Analysis:

C: 0.08%, Si: 0.01%, Mn: 0.25% P: 0.013%,  
S: 0.014%, Total N: 0.0023%, Cr: 0.010% in the rimmed layer and 0.051% in the core portion, soluble Al: 0.001% in the rimmed layer and 0.005% in the core portion.

Mechanical properties:

Yield point: 21.1 kg./mm.<sup>2</sup>,  
Tensile strength: 34.0 kg./mm.<sup>2</sup>,  
Elongation: 45.8%,  
Erickson value: 10.9 mm.  
Hardness: HRB 47.3

For comparison purposes, rimmed steel was produced from the same charge by the conventional method. After rimming action was effected for 25 minutes, a small lid was placed on the ingot mold.

Analysis of a cold-rolled sheet of 0.8 mm. thickness produced from the above comparison ingot and mechanical properties of the sheet, as annealed at 720°C. for three hours, are as follows:

## Analysis:

C: 0.04%, Si: 0.01%, Mn: 0.23%, P: 0.01%,  
S: 0.015%, Cr: 0.010% both in the rimmed and core portions,  
Soluble Al: 0.001% both in the rimmed and core portions.

Mechanical properties:

Yield point: 25.0 kg./mm.<sup>2</sup>,  
Tensile strength: 34.4 kg./mm.<sup>2</sup>,  
Elongation: 43.9%,  
Erickson value: 10.6 mm.  
Hardness: HRB 49.0

The microstructure of the cold-rolled sheet of the present invention, as annealed at 720°C. for 3 hours, heated for 3 minutes at 850°C., which is almost equal to the enameling firing temperature, and then quenched in salt water is shown in FIG. 6.

The results of tests for determining the practical usability of parts for gas cooking-pots for rice and gas ranges produced from the sheets of the present invention indicated no blister formation in any of the 130 parts.

What is claimed is:

1. A low-carbon steel ingot having an outer rimmed layer and an inner core layer, the ratio between said outer rimmed layer to the ingot thickness being between about 1:27 and 1:10 and the ratio between rimmed layer and core layer being about 3:70-1:20, the thickness of the rimmed layer being at least 0.05 mm., said core layer being alloyed with carbon-attraction inducing means for causing preferential attraction to carbon in the core layer, said means including at least one metal selected from the group consisting of Cr, Mn, Al, V and Ti in an amount of 0.1-0.2% for Cr and Mn, 0.15% for Ti and V, and 0.005-0.020% for Al, as soluble Al, and the content of said alloying metal in the core layer of said steel ingot being greater than that in the rimmed layer of the ingot by more than 0.05% for Cr and Mn, by more than 0.02% for Ti and V, and by more than 0.003% for Al as soluble Al, the rimmed layer containing not more than 0.02% C and the core layer containing 0.04-0.15% C.

2. Enameling grade steel sheets made from ingots having an outer rimmed layer containing not more than 0.02% C and an inner core layer containing from 0.04-0.15% C, the ratio of the thickness of the outer rimmed layer to the sheet thickness being about between 1:27 and 1:10, said core layer being alloyed with an austenite inducing agent for causing the steel with the agent to preferentially transform to austenite when heated to a given temperature as compared to said outer rimmed layer, said agent including at least one metal selected from the group consisting of Cr, Mn, Ti, V and Al in an amount of 0.1-0.27% for Cr and Mn 0.05-0.15% for Ti and V and 0.005-0.020% for Al, as soluble Al, and the content of said alloying metal in the core layer of said steel sheet being greater than that in the rimmed layer of said steel sheet by more than 0.05% for Cr and Mn, by more than 0.02% for Ti and V, and by more than 0.003% for Al, as soluble Al.

3. In a method of producing a steel ingot which comprises: pouring low-carbon molten steel into a mold, permitting the portion of the molten steel which is closest to the walls of the mold to solidify under rimming action until a peripheral rimmed portion is formed, the improvement which comprises introducing into the still liquid core portion of the steel mass an austenite inducing agent for causing the steel with the agent to preferentially transform to austenite as compared to the rimmed layer, said agent including at least one alloying metal selected from the group consisting of Cr, Mn, Al, V and Ti, in an amount between 0.1-0.2% for Cr and Mn, between about 0.05-0.15% for Ti and V, and between about 0.005-0.02% for

40 Al, as soluble Al, thereby obtaining a steel ingot having a rimmed layer and a core portion the ratio of thickness between said portions being about 3:70-1:20, said alloying elements being capable of preventing carbon migration toward the surface or of gathering carbon precipitating in the outer layer toward the core portion upon heating.

\* \* \* \* \*